

Patented Mar. 9, 1948

2,437,409

UNITED STATES PATENT OFFICE

2,437,409  
THE CITY OF ROCHESTER, NEW YORK  
ACTIVATING AND ELECTROPLATING  
STAINLESS STEEL

William M. Tucker, Rochester, N. Y., assignor to  
Eastman Kodak Company, Rochester, N. Y., a  
corporation of New Jersey

No Drawing. Application August 22, 1945.  
Serial No. 612,138

5 Claims. (Cl. 204—49)

This invention relates to electroplating, and more particularly to electroplating adherent electrodeposits of metals on alloys such as stainless steels and other alloys possessing a high order of corrosion resistance which is generally attributable to the presence of such alloying elements as chromium, nickel, columbium, and tungsten.

There are many instances where it is desired to plate copper, nickel and other metals on alloys containing the above-mentioned alloying metals. Various processes have been devised to reduce the corrosion resistance of these alloys and thereby to provide an active surface which will take an electrodeposit. Some such alloys may be suitably activated by either anodic and/or cathodic treatment in acid solutions of varying concentration.

Typical of such acid solution processes is cathodic activation in more than 30% by weight sulfuric acid, anodic activation in approximately 10% by weight hydrochloric acid and anodic processing in 25% by weight ortho phosphoric acid. The instant invention relates more directly, however, to the more passive types of alloys such as Type 302, 304, 309, 316, 317, 321, and 347 stainless steels, Hastelloys, Inconel, Worthite, Durimet, etc. These alloys may be suitably activated by comparatively high current density striking, or plating in highly acidic solutions of copper, or preferably nickel salts, containing considerable quantities of acids such as hydrochloric, phosphoric, sulfamic and sulfuric. The amount of acid employed in these processes tends to drop the efficiency of the metal deposition to less than 10%. Under such special circumstances it is possible to produce a satisfactory degree of surface activation on the normally passive alloy article to be plated. While such treatments satisfactorily activate the passive alloy surface, unfortunately the activated surface prevails only for a few minutes and it has been found that the passive film surface is automatically restored after this time. In the case of small articles, this self-restoration of the passive film may not interfere too much with the subsequent plating operation. However, when relatively large articles are activated, the deterioration of the active surface and the simultaneous partial or complete restoration of the passive surface frequently occurs before the article can be transferred to the plating bath and the plating operation com-

mensurate with the time required for the passive film to be restored.

STATEMENT OF THE INVENTION

The primary object of the invention is to provide a plating process for stainless steel articles which will produce an active surface which will remain active for a relatively long period of time.

Another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

Still another object of the invention is to provide a plating process for stainless steel articles which will produce an active surface which will remain active for a relatively long period of time.

The invention is presented in more detail in

the following examples which show typical processes for achieving excellent adhering electro-deposits on alloys which normally resist electro-plating and, therefore, cause poor or non-adhering deposits.

*Example I*

An article made of a chrome-steel alloy containing 18% chromium, 8% nickel and the balance iron together with small amounts of copper, manganese, tungsten, molybdenum, etc. was made the cathode in an electrolytic bath containing 32 oz./gal. of  $\text{NiCl}_2 \cdot 6\text{H}_2\text{O}$  and 16 oz./gal. of concentrated HCl (1.18 sp. gr.). An initial strike at a current of more than 200 amperes per square foot of cathode area for 2 minutes was employed followed by continuation of the striking process without current interruption at 25 to 30 amperes per square foot for 15 to 30 minutes. It was found that the alloy surface changed from a passive surface to an active surface and retained its activity for at least 10 minutes. This permits the operator to remove the article from the initial bath and properly install it in the subsequent bath where it received a permanent electrodeposit of nickel, according to the process shown in my U. S. Patent 2,147,415 of Feb. 14, 1939. The nickel plated on the alloy was found to have excellent adhesion and was in general satisfactory for most uses.

Where severe mechanical operations, such as drilling, turning, milling, etc. are contemplated and particularly when such operations will penetrate through the interphase between the deposit and the substrate metal, I prefer to supplement the above described process by a low temperature anneal at 400° F. to 1200° F. The low temperature anneal seems to enhance the resultant adhesion probably because it eliminates or reduces the strains resulting from adsorption or occlusion of atomic hydrogen originating in the prolonged striking operation.

*Example II*

A modification of the process described in Example I was tried in which the initial strike was conducted at a voltage yielding 100 amperes per square foot on the cathode for 2 to 4 minutes followed by continuation of the striking process without current interruption at 25 to 50 amperes per square foot for 15 to 30 minutes. The activated alloy was then installed in a nickel plating bath and plated in accordance with the directions given in my above mentioned Patent 2,147,415. An excellent appearing nickel layer was thus firmly electrodeposited on the alloy.

While I prefer to operate the electrodeposition according to the conditions set forth in the examples, I may employ  $\text{NiCl}_2 \cdot 6\text{H}_2\text{O}$  in amounts from 16 ounces per gallon to 48 ounces per gallon. The concentration of HCl may vary between 4 and 20 ounces per gallon. The initial high amperage per square foot employed in the process may be between 100 and 300 amperes for 2 to 4 minutes and the final lower amperage employed may be between 15 and 50 amperes per square foot of cathode area for 15 to 30 minutes.

When plating large pieces that require mechanical transfer from the strike bath to the subsequent plating bath and may take upwards of 10 minutes, the piece may be kept wet with cold water or a portion of the nickel strike solution so that the passive surface will not restore itself before the transfer is effected. It should be understood that deterioration of the active film will

occur even though the thin nickel strike film is on the alloy, after a relatively short period.

It will be understood by those skilled in the art that the piece to be plated is suitably degreased or otherwise cleaned as may be necessary before the strike operation. Such cleaning operations may include scouring with lime and acid or alkaline treatment to remove scale, etc.

The process thus described is applicable to all the alloys herein mentioned and after the nickel strike has been deposited on the alloy its active surface will also be receptive to copper or other metal plating as will be understood by those skilled in this art.

I claim:

1. The method of activating, and prolonging that activation, of the surface of stainless steel alloys having normally a passive surface which comprises making the alloy the cathode in an electrolytic bath composed essentially of nickel chloride and hydrochloric acid, electrolyzing the bath at a current of 100 to 300 amperes per square foot of cathode area for 2 to 4 minutes followed by a continuation of the electrolyzing at 15 to 50 amperes per square foot of cathode area for 15 to 30 minutes, whereby an active surface is established on the alloy which will persist for a substantially long period.

2. The method of activating, and prolonging that activation, of the surface of stainless steel alloys having normally a passive surface which comprises making the alloy the cathode in an electrolytic bath composed essentially of nickel chloride and hydrochloric acid electrolyzing the bath at 200 amperes per square foot of cathode area for 2 minutes followed by a continuation of the electrolyzing without current interruption at 25 to 50 amperes per square foot of cathode area for 15 minutes, whereby an active surface is established on the alloy which will persist for 10 minutes.

3. The method of activating and plating the surface of stainless steel alloys having normally a passive surface which comprises making the alloy the cathode in an electrolytic bath composed essentially of nickel chloride and hydrochloric acid, electrolyzing the bath at 100 to 300 amperes per square foot of cathode area for 2 to 4 minutes followed by a continuation of the electrolyzing at 15 to 50 amperes per square foot for 15 to 30 minutes, whereby an active surface is established on the alloy, and then increasing the plate thickness in a second plating bath before the active surface changes to a passive surface.

4. The method of activating and plating the surface of stainless steel alloys having normally a passive surface which comprises making the alloy the cathode in an electrolytic bath composed essentially of nickel chloride and hydrochloric acid electrolyzing the bath at 200 amperes per square foot of cathode area for 2 minutes followed by a continuation of the electrolyzing without current interruption at 25 to 50 amperes per square foot for 15 minutes, whereby an active surface is established on the alloy, and then increasing the plate thickness in a second plating bath before the active surface changes to a passive surface.

5. The method of activating and plating the surface of stainless steel alloys having normally a passive surface which comprises making the alloy the cathode in an electrolytic bath composed essentially of 32 ounces per gallon of  $\text{NiCl}_2 \cdot 6\text{H}_2\text{O}$  and 16 ounces per gallon of 1.18 specific gravity hydrochloric acid electrolyzing the

bath at from 100 to 200 amperes per square foot of cathode surface for 2 to 4 minutes followed by a continuation of the electrolyzing without current interruption at 25 to 50 amperes per square foot for 15 to 30 minutes, whereby an active surface is established on the alloy, and then increasing the plate thickness in a second plating bath before the active surface changes to a passive surface.

WILLIAM M. TUCKER.

#### REFERENCES CITED

The following references are of record in the file of this patent:

#### UNITED STATES PATENTS

| Number    | Name   | Date           |
|-----------|--------|----------------|
| 2,069,566 | Tuttle | Feb. 2, 1937   |
| 2,285,548 | Wesley | June 9, 1942   |
| 2,358,995 | Pinner | Sept. 26, 1944 |

#### OTHER REFERENCES

Transactions of the American Electrochemical Society, Apr. 1915, pages 144-154, vol. 27.